

June 15, 1926.

1,589,324

C. L. BEAL ET AL  
ELECTRODEPOSITION OF ORGANIC MATERIALS ON ANODES  
FROM AQUEOUS EMULSIONS THEREOF  
Filed May 7, 1925

FIG - 1.



FIG - 2.



FIG - 3.



Carl L. Beal and  
Leon W. Eberlin,  
INVENTORS,

BY *R. L. Stinchfield*

ATTORNEY.

Patented June 15, 1926.

## UNITED STATES PATENT OFFICE.

CARL L. BEAL AND LEON W. EBERLIN, OF ROCHESTER, NEW YORK, ASSIGNEES TO  
EASTMAN KODAK COMPANY, OF ROCHESTER, NEW YORK, A CORPORATION OF  
NEW YORK.

## ELECTRODEPOSITION OF ORGANIC MATERIALS ON ANODES FROM AQUEOUS EMULSIONS THEREOF.

Application filed May 7, 1925. Serial No. 28,690.

This invention relates to the electrodeposition of organic materials such, for instance, as rubber and cellulosic compounds, upon anodes from aqueous emulsions thereof.

- 5 One object of the invention is to provide an improved process of this nature which will minimize any harmful effects due to nascent oxygen liberated at the anode. Another object of the invention is to provide 10 such a process in which polarization by oxygen at the anode is counteracted. Still a further object of the invention is to provide a process in which the oxidized compounds formed at the anode will be compatible with 15 the substances deposited at that place. Other objects will hereinafter appear.

In the accompanying drawings, forming a part hereof, Figs. 1 to 3 are diagrammatic cross sections of different forms of apparatus which may be employed in carrying out our process.

In the electrodeposition of organic materials on anodes from aqueous emulsions thereof, such as aqueous emulsions of rubber or cellulosic compounds, like nitrocellulose, acetyl cellulose, and cellulose ether, the coatings sometimes become impaired by oxidation from nascent oxygen liberated at the anode when high current densities are employed. Moreover, under these conditions the process is apt to be slowed down by polarization at the anode, due to liberated oxygen. Of course, bubbles of oxygen tend to spoil the continuity and smoothness 35 of the deposit.

We have found that these difficulties can be wholly overcome or very largely avoided by having present in the anode zone, during the deposition, a metal which has a greater 40 affinity for nascent oxygen than the deposited organic material has. By the anode zone we mean the zone in which nascent oxygen is liberated; and by nascent oxygen we refer to electrolytically liberated atomic 45 oxygen which is known to be especially active. Examples of suitable metals are zinc, cadmium and magnesium. They are unusually effective when rubber is electrodeposited. Any of them will strongly 50 protect the rubber from injury by oxidation and will counteract polarization by combining with the oxygen at the anode. This results in few, if any, bubbles of oxygen to

impair the continuity and smoothness of the rubber deposit. Moreover, the oxides of 55 these metals, which are formed at the anode, are all compatible with the rubber and form useful fillers in the final composition.

We can have the desired metal, such as zinc, for example, in different forms at the anode 60 zone. For instance, the anode surface upon which the organic material is to be deposited may be coated with the metal, or the whole article upon which the anode surface is located, may be of the desired metal, such 65 as zinc or a zinc alloy. The metal may also be present in the droplets of the emulsion when the electrodeposition takes place. By way of illustration, we may prepare dispersions or emulsions of the desired metal with 70 the aid of protective colloids and combine them with the aqueous emulsions of organic materials such as rubber emulsions. Still a different way of bringing the metal to the 75 anode zone is to have it suspended in a porous or conducting coating over the surface upon which the deposit is to be made. Thus a mixture of gelatin and zinc powder 80 may be thinly painted over the electroconducting surface to be treated.

Our process may be used as an improvement upon or auxiliary to the electrodepositing processes disclosed in U. S. Patent No. 1,476,374, Samuel E. Sheppard and Leon W. Eberlin, Dec. 4, 1923, for electrodeposition of rubber coatings, and copending applications Serial No. 21,311, filed April 7, 1925, Leon W. Eberlin and Carl L. Beal, for electrodeposition of coatings of cellulosic compounds, and Serial No. 21,341, filed 90 April 7, 1925, Samuel E. Sheppard and Leon W. Eberlin, for electrodeposition of coatings comprising rubber and a cellulosic compound. Obviously the principle of our invention is adaptable to the production of 95 coatings wherever oxygen is liable to cause harm when electrodeposition takes place at an anode from aqueous emulsions or similar dispersions.

We shall now describe, by way of illustration, the preferred embodiment of our invention, but it will be understood that the latter is not limited to the details given, except as indicated in the appended claims.

We prefer to employ any of the rubber-containing emulsions disclosed in the above

cited patent and applications or in application Serial No. 611,162, Samuel E. Sheppard and Leon W. Eberlin, filed Jan. 6, 1923, for rubber emulsion and process of making the 5 same, and application Serial No. 21,840, Samuel E. Sheppard and Leon W. Eberlin, filed April 7, 1925, for aqueous emulsion of unvulcanized rubber and sulfur. The emulsions of the latter application are very de- 10 pendable in their properties.

The particles in all of the above mentioned emulsions act as if negatively charged, and travel toward the anode. Referring to Fig. 1, the electroconducting face 1 of the 15 object to be plated is covered with a thin layer or coating 7 of a suitable metal, such as zinc. This coating may be applied by any of the usual known or preferred zinc plating methods. The coated face is then 20 connected at 2 to anode line 3 so as to form the anode and is immersed in the emulsion 4. A suitable cathode is also placed in contact with the emulsion. For instance, the latter may be contained in a metal vessel 5 25 which is connected in the cathode circuit 6.

The current should preferably be an effectively unidirectional one. It may be a current of constant value or a direct current of pulsating character. In some instances it is 30 useful to employ an unbalanced alternating current, which is most conveniently obtained by superimposing an alternating current upon a direct current. The voltages and current densities to be employed can vary over 35 a considerable range. Higher current densities can be employed with greater safety because of the presence of our oxidizable metal in the anode zone. Since direct currents of 110 volts are conveniently available, 40 we prefer to use them and regulate the corresponding density to about  $\frac{1}{4}$  to  $\frac{1}{2}$  of an ampere per square inch of electrode surface to be coated. In general the plating expedients follow the practice given in the 45 patents hereinabove cited.

Referring to Fig. 2, the electroconducting surface 1 to be plated is part of a body composed wholly of zinc or zinc alloy. It is, therefore, ready to receive an electro- 50 deposited coating from aqueous emulsion of rubber 4, it being connected at 2 to anode line 3, vessel 5 being the cathode which is connected to line 6.

Referring to Fig. 3 the face 1, of the article to be plated, is coated with a substratum 55 17 composed of gelatin or glue carrying a powder or pigment of metallic zinc or magnesium. The substratum article is then connected at 2 to anode line 3 and is immersed in the electroconducting aqueous rubber emulsion 4. The vessel 5 may serve as a cathode and is connected to the cathode line 6. The use of a substratum for the production of an even coating is not claimed 60 herein, this being covered in the application 65

of Samuel E. Sheppard and Carl L. Beal, Serial No. 25,160, filed April 22, 1925, for electrodeposition of organic materials such as rubber and cellulosic compounds. In our present illustration the substratum not 70 only serves to insure an even coating, but serves as a vehicle for holding our oxidizable metal in the anode zone.

In all of the above examples, nascent oxygen is liberated as the anode and attacks the 75 metal much more rapidly than it does the rubber. Where the emulsion comprises natural latex, the final deposit has the least possible degradation, as is evidenced by its very high mechanical strength. It has no 80 degradation due to mechanical milling and little, if any, degradation due to chemical oxidation in the plating operations. Moreover, zinc oxide and magnesium oxide, (or 85 cadmium oxide if the latter rarer metal is used) are well known fillers for rubber compositions and, therefore, blend properly into the coating of rubber, even when the latter is vulcanized.

During the electrodeposition, particularly 90 with the arrangements illustrated in Figs. 1 and 2, the zinc, or equivalent metal, dissolves reversibly, that is electrolytically, and then combines with the oxygen. It is, therefore, not liable to passivity. 95

Having thus described our invention, what we claim as new and desire to secure by Letters Patent is:

1. The process of depositing organic material on an electroconducting surface of an 100 object, which comprises bringing said surface, connected as an anode, into contact with an aqueous electroconducting emulsion of said organic material and passing a depositing electric current through said surface and emulsion, there being present in the anode zone during the deposition a metal having a greater affinity for oxygen than 105 said organic material has.

2. The process of depositing rubber on 110 an electroconducting surface of an object, which comprises bringing said surface, as an anode, into contact with an aqueous electroconducting emulsion of rubber and passing a depositing electric current through 115 said surface and emulsion, there being present in the anode zone during the deposition a metal having a greater affinity for oxygen than rubber has, and the oxide of said metal being compatible with rubber in the deposit. 120

3. The process of depositing organic material on an electroconducting surface of an object, which comprises bringing said surface, connected as an anode, into contact with an aqueous electroconducting emulsion 125 of said organic material and passing a depositing electric current through said surface and emulsion, there being present in the anode zone during the deposition sufficient zinc to take up liberated oxygen. 130

4. The process of depositing rubber on an electroconducting surface of an object, which comprises bringing said surface, as an anode, into contact with an aqueous electroconducting rubber emulsion and passing a depositing electric current through said surface and emulsion, there being sufficient zinc in the anode zone during the deposition to take up liberated oxygen.
5. The process of depositing organic material on an electroconducting surface of an object, which comprises covering said surface with a layer of a metal which has a greater affinity for oxygen than said organic material has, bringing said covered surface into contact with an aqueous electroconducting emulsion of said organic material and passing a depositing electric current through said surface, covering and emulsion.
- 10 6. The process of depositing rubber on an electroconducting surface of an object, which comprises covering said surface with a metal having a greater affinity for oxygen than rubber has, which counteracts polarization at the anode, bringing said covered surface into contact with an aqueous electroconducting rubber emulsion and passing a depositing electric current through said surface, covering and emulsion. 25
7. The process of depositing rubber on an electroconducting surface of an object, which comprises covering said surface with zinc, bringing said covered surface into contact with an aqueous electroconducting rubber emulsion and passing a depositing 30 electric current through said surface, zinc covering and emulsion. 35

Signed at Rochester, New York, this 4th day of May 1925.

CARL L. BEAL.  
LEON W. EBERLIN.